

Patented May 12, 1925.

1,537,752

# UNITED STATES PATENT OFFICE.

FRANK H. COYNE, OF BRYN MAWR, PENNSYLVANIA; FRANCES MOFFETT COYNE  
EXECUTRIX OF SAID FRANK H. COYNE, DECEASED.

## ART OF PRODUCING WATERPROOF SHEETS FROM FIBROUS MATERIAL BY THE USE OF SULPHUR.

No Drawing.

Application filed March 8, 1919. Serial No. 281,465.

*To all whom it may concern:*

Be it known that I, FRANK H. COYNE, a citizen of the United States, and a resident of Bryn Mawr, in the county of Montgomery and State of Pennsylvania, have invented an Improvement in Art of Producing Waterproof Sheets from Fibrous Material by the Use of Sulphur, of which the following is a specification.

- 10 My invention has relation to a method of using sulphur as an adhesive in uniting objects or fabrics, and to the composite object or fabric thus produced, with the purpose of giving to such composite objects or 15 fabrics or objects produced therefrom, liquid proof and moisture proof and other desirable qualities. My invention also includes the composite object and fabric thus produced.
- 20 This process is particularly applicable to uniting sheets of material, such as sheets of paper, veneer, or other materials used in building up laminated objects or materials.

- 25 I effect the result indicated by introducing my sulphur between the articles or sheets to be united, when the sulphur is in a peculiar condition.

Sulphur occurs crystallized in yellow 30 transparent crystals in the form of rhombic octahedra. It, however, occurs in several physical and molecular forms when subjected to the influence of heat. It becomes thick and viscous, treacly or plastic at temperatures ranging from 320° F. to 838° F., 35 when it boils. It is known that if sulphur, when in this thickened condition, be suddenly greatly lowered in temperature, as by pouring a small stream or film into cold 40 water, or by subjecting a thin film or ribbon-like mass to other sudden chilling effect, it is converted into a soft mass resembling caoutchouc.

This form is not permanent, but after a 45 length of time, depending upon the bulk and other conditions, the sulphur assumes a rigid state. It is at this point that my discovery comes in.

The object of my invention is to produce 50 a more homogeneous product than heretofore, as far as I am aware, has been produced, also to produce one which is more nearly completely water-proof than such

products as heretofore manufactured and also to cheapen the cost of production.

I have discovered that under certain conditions as to temperature and method of application, sulphur may be employed as an adhesive for the purpose of securing together two or more sheets of fibrous material to thereby produce a laminated sheet of such material.

My invention has other objects and advantages which will be pointed out in the detailed description thereof which follows or will be apparent from such description.

I have discovered that sulphur, when in a molten state, may be employed as an adhesive to secure together sheets of fibrous or other material. When employing the sulphur as an adhesive, my experience has been that it should be raised to a temperature well above its lowest fusion point. My experience indicates that preferably such temperature should be not less than approximately 300° F.

It is desirable to employ the adhesive (sulphur) when its adhesive quality is at the highest. The adhesive, sulphur, may be used to unite the plies of a composite sheet, applied when in the condition indicated, or the peculiarity in question may be induced by the use of heat after the application of sulphur in powdered or other substantially non-adherent condition. The temperature at this point is too high for the fiber to stand long. If the super-melted sulphur be used and distributed in any of the well known ways, it is in condition immediately upon contact with the surface of the sheet to be coated and adheres to it. A second sheet is immediately and as nearly simultaneously as possible, applied in turn to the sticky adhesive coating so that the two sheets are immediately stuck together by a sticky, tough coherent and temporarily flexible, plastic coating.

It may be shaped while in this condition. That is to say the composite sheet, or laminated material, may be bent, or rolled, up etc. according to the flexibility, or pliability, of its constituent sheets other than their interposed layer of, at that stage, plastic, or flexible, sulphur, for example the composite sheet in its thus flexible condition may be shaped from flat into tubular, or cylindrical, contour with-

55

60

65

70

75

80

85

90

95

100

105

out displacing, or impairing the cohesion of, its constituents; the sulphur, like other substances in a viscous, or mobile, liquid condition, then possessing in itself the quality of flexibility, or plasticity, and, to an extent, also imparting the same to the sheets of other material constituting the composite, or laminated, article of which the sulphur forms a material part.

10. After the sulphur in my complex product has hardened, or set, its flexibility and plasticity, and, to a degree, of the article, or laminated composite sheet, of which it forms a part, may, whenever, and as long as desired for special purposes, be restored, as, for example, by heating to an above referred to temperature and again quickly cooling, thus substantially reutilizing, in that way and to that extent, a characteristic feature of my above described invention. Thus, in all cases there is a period, or stage, during which my novel complex sulphur-cemented article, or product, is usefully flexible or plastic, or, after it has hardened, capable of being again made flexible or plastic, and again relatively rigid or unbending by aid of my invention, and I therefore believe that its said products, the sulphur of which has hardened or set, are, as well as the therein sulphur, properly definable as being latently plastic; that is to say possessing the property of becoming indefinitely alternately flexible or the reverse without permanent loss, or modification, of their other normal characteristics or qualities.

I do not, however, desire to limit my invention to the use of sulphur at a temperature greater than 300° F., because it may be found that under some circumstances and conditions it may be practicable to employ it as an adhesive at a substantially lower temperature.

In the employment of sulphur as an adhesive according to my invention, it is placed in a suitable receptacle and raised to a temperature such as above indicated, and by known means is applied to the surface or surfaces of sheets to be secured together. After the sulphur, which may be in a viscous or a mobile liquid condition, is applied to the surface or surfaces of the sheets to be secured together, such surfaces are placed in contact with each other and are pressed together. The sulphur quickly sets and hardens and constitutes not only an efficient adhesive for connecting the sheets together, but also constitutes a water and moisture proof layer for preventing the passage of water or moisture through the laminated sheet formed by the joining together of two or more sheets.

I have been unable to determine within a degree of certainty why it is that when sulphur is applied at a temperature much

above its lowest fusion point and while it is in a viscous or liquid condition, it acts as an efficient adhesive, particularly in the securing together of fibrous sheets, but believe that it may be due to the fact that upon the application of the sulphur at the relatively high temperature suggested, it is quickly cooled, and as the temperature is lowered it reaches a point at which the layer of sulphur is in a thoroughly liquid state, in which condition it combines with and adheres to the adjacent surfaces of the sheets to be connected. Further cooling to a temperature below its lowest fusion point quickly takes place so that the layer of sulphur is hardened and constitutes an efficient binding agent or adheres as above described.

I claim:

1. The process of making a laminated paper structure which consists in moving a layer of paper over a support, applying to said layer, while it is moving over the said support, sulphur previously heated until it reaches a temporarily viscous adhesive condition and while the sulphur is still in its adhesive condition applying a second sheet and subjecting said sheets after sulphur has been applied and they are stuck together to conditions which transform them into an elastic and temporarily flexible fabric.

2. As a new article of manufacture, a fabric consisting of layers of material having between them layers of sulphur, the layers of sulphur procured between said layers of material in adhesive condition, said fabric being liquid and moisture-proof, and normally stiff but latently plastic.

3. The new article of manufacture which comprises a plurality of mutually parallel layers or sheets of paper material which are held together by a substantially co-extensive, latently plastic, layer or sheet composed essentially of sulphur interposed between, to an extent combined with, and adherent to, the respectively mutually opposite areas of first mentioned layers or sheets.

4. The process of making a laminated sheet which consists in procuring between successive layers of paper, layers of sulphur in viscous condition, effecting quick chilling of said sulphur to adherent condition and applying pressure to distribute the sulphur between the sheets and to force it into intimate adherent relation to the fibers of the paper.

5. The process which consists in juxtaposing alternate layers of sulphur heated to viscosity, and of organic, fibrous material, chilling the sulphur to adhesive condition, before the fibrous material becomes prohibitively heated, and compressing the layers.

6. The method of uniting sheets of paper material which comprises interposing sulphur in viscous state between them and causing it to adhere to the therewith respectively contacting sheets.

7. The new composite article of manufacture, comprising unitary sheets of paper material combined together by intervening

sulphur in the form of a continuous, water and moisture-proof, layer composed of co-<sup>10</sup> fused mutually co-adherent particles of sulphur.

In testimony that I claim the foregoing as my invention I have hereunto set my hand this 27 day of January, A. D., 1919.

FRANK H. COYNE.